

## UNITED STATES PATENT OFFICE

2,179,239

## COLOR PHOTOGRAPHY

Gustav Wilmanns, Wolfen, Kreis Bitterfeld, Wilhelm Schneider, Dessau, and Ernst Bauer, Hersbruck, Mfr., Germany, assignors, by mesne assignments, to Agfa AnSCO Corporation, Binghamton, N. Y., a corporation of Delaware

No Drawing. Application November 13, 1937, Serial No. 174,350. In Germany April 10, 1935

5 Claims. (CL 95—6)

Our present invention relates to color photography and more particularly to a process and material in which color is produced in a colloidal emulsion layer by the action of an oxidation product of a photographic developer on a dyestuff component incorporated in said layer.

This process of color forming development has first been disclosed in U. S. Patents 1,102,028 and 1,055,155 to Fischer.

10 If a photographic emulsion layer containing these dyestuff components is developed by means of a developer containing free amino groups, for instance phenylene-diamines, especially the mono- or unsymmetrically disubstituted ones like 15 p-dimethylaminoaniline, ethoxy-p-dimethylaminoaniline, there is obtained a colored photographic picture.

The color of the pictures depends upon the dyestuff forming components applied to the layer. 20 Pyrazolones for instance yield blue-red dyes, derivatives of acetoacetic ester yield yellow colorings, and naphthols yield blue colors.

The dyestuff components of Fischer, however, merely lent themselves to the production of pictures in one single color. When dyestuff components which yield various colors by development were incorporated in several superposed layers it became apparent after developing that the components had diffused into all the other 25 layers, viz., that a separation of the color values of the photographed object had not been achieved. Even if components were selected from those listed in the aforementioned patents which are difficultly soluble, i. e., which are capable 30 of being incorporated in the layers in the form of an insoluble precipitate, these components did not show a satisfactory fastness to diffusion, unless they were entirely insoluble, in which case 35 they did not react at all with the developers and merely a black silver picture was produced.

Even for the production of single-colored reversal pictures the dyestuff components were useless inasmuch as they were washed out of the layers during the black-and-white development, 45 so that for the subsequent color development an insufficient amount of them remained in the layers, or at least they were apt to diffuse into the developer itself thereby soiling pictures which were simultaneously developed in another color. 50 It is therefore an object of the present invention to provide a material in which all these disadvantages and drawbacks are overcome.

A further object is to provide a process by which dyestuff components may be obtained 55 which are soluble in aqueous liquids and which

are fast to diffusion once they are incorporated in the photographic emulsion layers.

A further object is to provide dyestuff components which will not be removed from their respective photographic layers by the action of aqueous alkaline liquids such as for instance developing solutions.

A further object of the invention is to provide a color photographic multi-layer material comprising a series of superposed emulsion layers, each layer containing a dyestuff component of the above described kind.

Further objects will be apparent from the detailed specification following hereafter.

This application is to be regarded as a continuation in part of our copending application Ser. No. 72,718 filed April 4, 1936.

The invention is based on the observation that by adding groups to the coupling components having so large a number of atoms that the resultant molecule is substantially increased in size, the dyestuff components, while retaining their solubility in aqueous liquids, do not tend to diffuse from the photographic emulsion layer or into the developing solution.

As dyestuff components which may be substituted by radicals which will increase their molecular size the following may be named by way of example:

All compounds with an active methylene group, for instance acetoacetic ester, bromacetoacetic ester, acetoacetic anilide, cyanoacetic ester, benzoylacetoacetic ester, benzoylacetic acid anilide, terephthaloylacetic ester, hydrindenes such as for instance diketohydrindene, pyrazolones such as for instance 1-phenyl-3-methyl-pyrazolone, 1-phenyl-3-phenyl-pyrazolone, coumaranone, malonic acid anilide, omega-cyanoacetophenone, hydroxythionaphthene etc. There are further used phenols such as for example meta-amino-phenol, o-o'-dinaphthol, o-hydroxydiphenyl, o-6-dihydroxydiphenyl, substituted naphthols as for instance  $\alpha$ -naphthol, dinaphthol, 1,5-hydroxy-naphthol, chloronaphthol and trichloronaphthol, substituted aminonaphthols, for instance 1,5-aminonaphthol, phenolcarboxylic acids, for instance salicylic acid, naphthol carboxylic acids, for instance  $\alpha$ -hydroxynaphthoic acid. Of the benzene and naphthalene derivatives those hydroxy compounds are especially suitable which in p-position to the hydroxy group have either no substituent at all or a negative substituent such as for instance chlorine, sulfonic acid. Also other substitution products of the above named

compounds may be used, such as for instance nitro derivatives.

It is impossible to define a general chemical structure of the radicals which are to be introduced into the molecule of the aforementioned coupling components. However, it should be generally stated that all organic radicals which produce a substantial increase in the molecular size of the dyestuff components are suitable for the purpose of the present invention. The exact size of the radicals which are to be introduced depends largely upon the tendency of diffusion which the substituted dyestuff component possesses. Thus radicals from 5 carbon atoms upwards will be very useful in some cases, while in others radicals of at least 12 to 18 carbon atoms are required.

The carbon atoms may be arranged in chain or nuclear formation and they may be linked to hydrogen or other atoms, such as oxygen, sulfur, selenium, nitrogen and halogen etc. These radicals may in themselves have the structure of the aforementioned dyestuff components so that dyestuff components which are obtained by linkage of several molecules of coupling components are also within the scope of the present invention.

For the synthesis of these compounds it is advisable to introduce the radicals which impart the fastness to diffusion to the molecule of the dyestuff forming component by means of an amino, carboxyl, or hydroxyl group in the form of an amide or an ester. However, a direct connection by means of C-C-linkage of coupling component and the radical to be introduced is also possible. Also Schiff's bases may be formed. In order to increase the solubility of the compounds they may contain special groups imparting solubility to them as for instance carboxyl or sulfo-groups.

For the production of photographic layers, especially those dyestuff components will be suited which may be introduced into the layer in a dissolved state. It has been found that in the manner suggested above components may be obtained which possess a satisfactory fastness to diffusion in dilute alkaline solutions and which are soluble in aqueous liquids in some cases by addition of slight quantities of an organic solvent, so as to be easily incorporated in photographic layers in a dissolved state. Of course there always exists the possibility of introducing the undissolved dyestuff components into the layer, but such layers yield less clear pictures and pictures of coarser grain.

Of the great number of groups which come into question for the production of dyestuff components fast to diffusion some have been found to be especially suitable. Such groups are for instance the substantive groups with which direct cotton dyestuffs of good qualities of fastness could be obtained. Chemically these are groups which contain a comparatively long chain of conjugated double bonds, such as for instance diphenyl, dianisidine, tolidine, diphenyl-carboxylic acid, 3-hydroxy-4-diphenyl-carboxylic acid, diaminobenzoylaminodiphenyl, 2,2'-dihydroxy-4,4'-diamino-diphenyl, stilbene, diaminostilbene, diaminobenzoylaminostilbene, azoxybenzene, hydroxynaphthoic acid, for instance 2,3-hydroxynaphthoic acid, 4,2',3'-hydroxynaphthoylaminocaniline, diaryl ureas, as for instance diaminodiphenylurea, diaminobenzoylaminodiphenylurea, the carbamide of aminobenzoyl-

amino-o-sulfanilic acid, heterocyclic nuclei as for example triazines, thiazoles, benzthiazoles, dehydrothiotoluidines, oxazoles, nuclear cyanuric derivatives in which several dyestuff components are linked by means of the cyanuric nucleus and which may contain still further substantive groups, furthermore certain aminonaphthols as for instance 2-amino-5-naphthol-7-sulfonic acid and 2-aminobenzoylamin-5-naphthol-sulfonic acid, furthermore highly molecular compounds as terephthaloyl bisacetic ester, 2,3-hydroxyanthracene carboxylic acid, 2,3-hydroxycarbazole carboxylic acid, aminochrysene, aminopyrene, aminonaphthyleneoxide.

The compounds obtained in this manner may be dissolved in alkali with perhaps an addition of alcohol or other organic solvents and may then be added to layer forming colloids without any precipitation. The fastness to diffusion of these components may further be increased by the introduction into their molecule of still further groups which increase their molecular size, such as for instance benzoyl and benzoylamin radicals or by means of a precipitating compound, such as for instance diphenyl guanidine.

As a binding agent for the photographic layers especially gelatin is used, however, all the other colloids which are usually employed in photographic practice may be used.

The following examples serve to illustrate the invention:

1. 2 mols of salicyclic acid chloride is condensed with 1 mol of diaminostilbene in pyridine. There is obtained a component of the following formula:



8 grams of the resulting compound are dissolved in 3 cc. of sodium hydroxide of 40 per cent strength, 25 cc. of methanol, and 70 cc. of water and then added to 500 cc. of a gelatin emulsion of 5 per cent strength. By developing with p-diethylaminoaniline a blue picture is obtained.

2. From salicyclic acid chloride and benzidine a dyestuff component of the following formula is obtained:



There are added to the component 9 grams of salicyclic acid chloride dissolved in the same manner as in Example 1 and 500 cc. of a 5 per cent emulsion. By developing with p-diethylaminoaniline a blue picture is obtained.

3. From dehydrothiotoluidine and  $\alpha$ -hydroxy-naphthoic acid chloride the following component is obtained:



5 grams of this compound are dissolved as described in Example 1 and added to a 5 per cent gelatin emulsion. By developing with a color forming developer a blue picture is obtained.

4. From dehydrothiotoluidine and salicylic

5

10

15

20

25

30

35

40

45

50

55

60

65

70

75

acid chloride the following compound, which yields a blue picture, is obtained:



10 5. A component yielding a blue picture and having the formula:



20 may be obtained from 7-p'-aminophenyl-5-methyloxazole and hydroxynaphthoic acid chloride.



30 6. A component yielding a red picture and having the formula:



40 is obtained from the hydrazine of the dehydrothiotoluidine which is condensed with p-nitrobenzoylactic ester, then reduced and again condensed with benzoylchloride. The compound is dissolved as described in Example 1.

45 7. A dyestuff component yielding a red picture and having the formula:



55 45 is obtained in analogous manner as in the preceding example with the sole exception that the last process step consists in condensing with diphenylcarboxylic acid chloride instead of with benzoylchloride.

60 50 8. A dyestuff component yielding a red picture and having the formula:



65 is obtained from the hydrazine of the 2-p'-amino-5-methylbenzoxazole which is condensed with p-nitrobenzoylactic ester, whereas the nitro group is reduced to the amino group and the latter reacted with diphenyl-dicarboxylic acid chloride.

70 9. A dyestuff component yielding a yellow picture and having the formula:



is obtained by heating 2 mols of benzoylacetic ester and 1 mol of benzidine. 3 grams of the compound are dissolved according to the prescriptions given in Example 1 and added to 500 cc. of a 5 per cent gelatin emulsion.

10. A compound of the formula



15 yields when developed with color forming developers a yellow picture. The compound is obtained by heating 2 mols of benzoyl-acetic ester and di-p-aminophenylurea in boiling zylene while at the same time distilling off the formed alcohol.

20 11. A compound of the formula



25 is obtained by condensing hydroxydiphenylcarboxylic acid chloride and 2,2'-dihydroxy-4,4'-diaminodiphenyl. By development with color forming developers the compound yields a blue picture.

30 What we claim is:

35 1. A photographic emulsion layer having incorporated therein a color forming development component having linked to an atom of its molecule a substantive grouping of so large a number of carbon atoms that the molecular size of said component is materially increased, said grouping being capable of rendering said component fast to diffusion.

40 2. A photographic emulsion layer having incorporated therein a color forming development

45 component having linked to an atom of its molecule the diphenyl grouping, said grouping being capable of rendering said component fast to diffusion.

50 3. A photographic emulsion layer having incorporated therein a color forming development component having linked to an atom of its mole-

55 cule the stilbene grouping, said grouping being capable of rendering said component fast to diffusion.

60 4. A photographic emulsion layer having incorporated therein a color forming development component having linked to an atom of its molecule the benzothiazole grouping, said grouping being capable of rendering said component fast to diffusion.

65 5. A photographic silver halide-gelatine emulsion layer having incorporated therein a color forming development component having linked

to an atom of its molecule a group of so large a number of atoms that the molecular size of said component is more than doubled, said component although soluble in aqueous photographic developing solutions being as a result of its molecular size incapable in such dissolved form of

diffusing in gelatine in any photographic treating bath.

GUSTAV WILMANNS.  
WILHELM SCHNEIDER.  
ERNST BAUER.